

1

3,168,400

## RAPID PROCESSING OF PHOTOGRAPHIC COLOR MATERIALS

John Blackmer and Howard W. Vogt, both of Rochester, N.Y., assignors to Eastman Kodak Company, Rochester, N.Y., a corporation of New Jersey  
 No Drawing. Filed May 22, 1961, Ser. No. 111,489  
 12 Claims. (Cl. 96—22)

This invention relates to photography, and more particularly, a method for increasing the speed of processing photographic films and papers for recording photographic images in color.

In multi-layer photographic elements used for color photography, there are usually at least three selectively sensitive emulsion layers coated on one side of a photographic support, such as film or paper. One of the silver halide emulsions is usually selectively sensitized to the red region of the spectrum, another to the green and the third to the blue region of the spectrum. In color materials for reversal processing, there is usually a yellow filter layer between the support and the conventional uppermost blue-sensitive layer. The red- and green-sensitive layers generally lie between the yellow filter layer and the support. Such color materials may be designed for processing in photographic developers containing a color coupler or color-forming compound, which couples with the oxidation products of the color developer to provide the desired color image. Other photographic materials are designed in such a fashion that the coupler is incorporated in the silver halide emulsion layer itself, or in a layer contiguous thereto. Such modifications are well known to those skilled in the art, and it is to be understood that the present invention is concerned both with photographic elements which are designed to be processed in color developers containing the couplers or color materials which contain the couplers in the silver halide emulsions, or in layers contiguous thereto. Multi-layer materials of the type which can be employed in the present invention have been previously described in the prior art, such as Jelley and Vittum U.S. Patent 2,322,027, issued June 15, 1943, and Mannes et al. U.S. Patent 2,252,718, issued August 19, 1941.

It is known that photographic silver halide emulsions can be processed at elevated temperatures, thereby materially shortening the processing time. However, as the temperature of the processing solutions is raised, the photographic layers conventionally used suffer the serious disadvantage of softening, which causes offsetting of the layers and reticulation from the supporting surface, such as film or paper. Attempts have been made to overcome this softening difficulty by treatment of the photographic element prior to processing with an aqueous solution containing a hardener for the conventional hydrophilic colloid layers which generally contain gelatin or some similar material. Aldehydes, such as formaldehyde, glyoxal, succinaldehyde, glutaraldehyde, etc., have been proposed for this purpose, but it has been found that even small amounts of these aldehydes will carry through into one or more of the color developers and react with the color couplers, thus causing serious difficulties.

We have now found a novel method which permits high temperature processing by use of a prebath containing a hardening agent for the hydrophilic colloid and at the same time avoids the substantial difficulties previously experienced by carrythrough of the hardening agent of one of the subsequent processing baths, such as the color developer, where the hardening agent has deleterious side reactions leading to the formation of sludge and scum. According to our process, the aforementioned difficulties are avoided by using an aqueous bath, after the hardening bath, which contains an amine which reacts with the re-

2

sidual hardening agent, such as aldehyde, thereby preventing carrythrough into one of the subsequent treating baths. Using this technique, it has been found possible to shorten the processing time of a conventional incorporated coupler film from approximately 52 minutes by conventional processing to about 19 minutes, while providing quality substantially equal to that obtainable using prolonged processing conditions.

The prebaths used in our invention following the aldehyde hardening bath comprise an aqueous solution containing at least one primary amine compound containing in addition to the -NH<sub>2</sub> group a hydroxyl group, a carbonyl group, or an amino group, which may have a substituent thereon. The concentration of the amine compound in the prebath can be varied, depending upon the amount of aldehyde which carries over from the aldehyde hardening bath. In general, we have found that from about 1 gram to about 100 grams per liter of amine compound is sufficient to remove substantially all traces of aldehyde from the emulsion layers, so that aldehyde is not released into one of the subsequent processing baths. The amine compounds, useful in our invention, can be employed in the form of their free bases, or they can be employed in the form of their water-soluble acid addition salts, such as the hydrochloride, sulfate, phosphate, etc. Amine compounds which can be usefully employed in our invention comprise the following:

|     |                                                                                                                   |
|-----|-------------------------------------------------------------------------------------------------------------------|
| (1) | H <sub>2</sub> N—OH                                                                                               |
| 30  | Hydroxylamine                                                                                                     |
| (2) | $\begin{array}{c} \text{O} \\ \parallel \\ \text{H}_2\text{NNHCONH}_2 \end{array}$                                |
| 35  | Semicarbazide                                                                                                     |
| (3) | H <sub>2</sub> NNH <sub>2</sub>                                                                                   |
| 40  | Hydrazine                                                                                                         |
| (4) | $\begin{array}{c} \text{O} \\ \parallel \\ \text{H}_2\text{NNHCNHNH}_2 \end{array}$                               |
| 45  | Carbohydrazide                                                                                                    |
| (5) | $\begin{array}{c} \text{O} \quad \text{O} \\ \parallel \quad \parallel \\ \text{H}_2\text{NCNHCNH}_2 \end{array}$ |
| 50  | Biuret                                                                                                            |
| (6) | $\begin{array}{c} \text{NH} \\ \parallel \\ \text{H}_2\text{NNHCNHNH}_2 \end{array}$                              |
| 55  | Aminoguanidine                                                                                                    |
| (7) | $\begin{array}{c} \text{O} \\ \parallel \\ \text{H}_2\text{NNHCNHNCH}_3 \end{array}$                              |
| 60  | Methylsemicarbazide                                                                                               |
| (8) | $\begin{array}{c} \text{O} \\ \parallel \\ (\text{CH}_3)_3\text{NCH}_2\text{CONHNH}_2\text{Cl}^- \end{array}$     |
| 65  | Girard's reagent                                                                                                  |

In preparing the amine-containing prebath compositions useful in the present invention, it is the usual practice to dissolve one of the amine compounds in water, and then adjust the pH of the treating solution so that a pH within the range of about 4.5 to about 8.0 is obtained. Improved reaction of the amine compound with the aldehyde contaminants in the emulsion layers generally occurs more rapidly at a pH below 8.0. Higher pH levels can sometimes be used, although prolonged contact times may be required in order to compensate for the lower rate of reaction.

The most advantageous concentration of amine compound for a particular processing run can be determined by developing a series of test strips of photographic multi-layer elements wherein the concentration of the amine compound, as well as the concentration of the

aldehyde in the hardening bath, are varied. The rate of reactivity of the amine-containing composition can be varied by variation of the pH as mentioned above. Advantageously, the pH can be varied by the addition of an alkaline solution, such as one containing sodium carbonate, potassium carbonate, sodium hydroxide, etc., or by the addition of an aqueous acidic solution, such as a solution of acetic acid, hydrochloric acid, sulfuric acid, etc. If desired, a buffer, such as sodium acetate, can be added to maintain the pH at a relatively constant level.

The photosensitive layers present in the photographic elements processed according to our invention can contain any of the conventional silver halides as the photosensitive material, and it is to be understood that our invention is not concerned with the chemical nature of these ingredients. Silver halide emulsions, such as silver chloride, silver bromoiodide, etc., can be usefully employed, although other silver halide emulsions can be employed to equal advantage. Any of the conventional photographic supports can be used to serve as a carrier for the silver halide films. Glass, cellulose ester film, etc., can be employed.

The concentration of aldehyde in the aldehyde hardening bath can be varied, depending upon the processing temperature and the like. Sufficient aldehyde is generally employed to prevent any substantial softening at elevated temperatures lying between about 85° F. and 150° F. The concentration of aldehyde will obviously depend upon the hardening property of a particular aldehyde, some aldehydes being more reactive with the hydrophilic colloid, such as gelatin or polyvinyl alcohol.

The process of our invention can be used in the treatment of photographic color elements designed for reversal color processing, or in the processing of negative color materials, or color print materials. The important feature of our invention is the use of an aqueous solution containing an amine compound of the above type after treatment of the photographic element with an aldehyde hardening bath, but prior to photographic development. This technique avoids substantial carry-over of any aldehyde compound into one of the subsequent treating baths where its presence might cause deleterious effects. Washing with water following an aldehyde hardening bath does not remove sufficient aldehyde to prevent the difficulties which have been mentioned above. However, simple treatment with an aqueous solution of one of the amine compounds of our invention removes the aldehyde and even reduces the number of washing steps with water which have been previously employed in commercial processing of many photographic elements. If the concentration of amine compound is relatively high so that some of this compound carries over into one of the subsequent treating baths, this does not cause any serious difficulties. It has been found that many of these compounds have useful properties even in the subsequent treating baths. For example, where 20 grams per liter of succinaldehyde were employed in a hardening bath to permit high temperature processing, it was found that the useful concentration of hydroxylamine (or a salt thereof) should be about 50 grams per liter, although higher amounts had no deleterious effect upon photographic quality.

Following treatment of the hardened element in the prebath, the element can thereafter be processed in a normal sequence using conventional processing solutions and techniques, or in other cases, the process can be adapted to other processing techniques, such as surface-layer processing of the type described in the copending application of Turner and Wilson, Serial No. 87,874, filed February 8, 1961.

The following example will serve to illustrate the simple technique of avoiding the difficulties previously experienced in processing hardened photographic elements at elevated temperatures.

## Example

A three-color silver bromoiodide film, wherein gelatin was employed as the hydrophilic colloid and wherein cyan, magenta and yellow color formers of the type described in the Jelley and Vittum patent mentioned above were incorporated in the emulsions, was exposed for  $\frac{1}{50}$  second to a 500-watt tungsten lamp, adjusted to a color temperature of 6100° K. in an intensity scale sensitometer. The exposed strip was then treated for 2 minutes in a hardening bath at 100° F. having the following composition:

|                        | Grams |
|------------------------|-------|
| Succinaldehyde         | 10    |
| Sodium acetate         | 10    |
| Water to make 1 liter. |       |

Without any intermediate water wash, the film was immersed for 30 seconds at 100° F. in an amine-containing bath having the following composition:

|                          | Grams |
|--------------------------|-------|
| Sodium hexametaphosphate | 0.5   |
| Hydroxylamine            | 25    |
| Sodium bromide           | 1.0   |
| Sodium sulfate           | 50    |
| Water to make 1 liter.   |       |

The treated film was then developed for 3 minutes at 100° F. in a black-and-white negative developer, such as one having the following composition:

|                                                    |       |      |
|----------------------------------------------------|-------|------|
| Water, 90° F. (32° C.)                             | liter | 1.0  |
| Sodium hexametaphosphate                           | grams | 2.0  |
| N-methyl-p-aminophenol sulfate                     | do    | 6.0  |
| Sodium sulfite, desiccated                         | do    | 50.0 |
| Hydroquinone                                       | do    | 6.0  |
| Sodium carbonate, monohydrate                      | do    | 35.0 |
| Potassium bromide                                  | do    | 2.0  |
| Sodium thiocyanate                                 | do    | 1.5  |
| 6.5% solution of 6-nitrobenzimidazole nitrate ccs. | 12.0  |      |
| 0.1% solution of potassium iodide                  | ccs   | 10.0 |

At this point it was possible to omit the conventional water wash and first-hardener treatment and to proceed with treatment for 30 seconds in an acid rinse bath having the following formula.

## Acid rinse:

|                     |       |               |
|---------------------|-------|---------------|
| Water               | ml    | 800           |
| Glacial acetic acid | ml    | 30.0          |
| Sodium hydroxide    | g     | 1.75          |
| Water to            | liter | 1             |
| pH at 80° F.        |       | 3.8 $\pm$ .40 |

The film was then washed for 30 seconds in water at 100° F. and then given either a flash exposure to strong white light or a chemical exposure in a reducing bath, such as aqueous alkaline bath containing potassium borohydride. (See Henn, Bulloch and Bard U.S. application Serial No. 699,478, filed November 29, 1957, now U.S. Patent 2,984,567, issued May 16, 1961.) The film was then developed for 3 minutes at 100° F. in a color developer having the following formula:

|                                                                                |       |       |
|--------------------------------------------------------------------------------|-------|-------|
| Water, 70° to 80° F. (21° to 27° C.)                                           | liter | 1.00  |
| Benzyl alcohol                                                                 | cc    | 6.0   |
| Sodium hexametaphosphate                                                       | gm    | 2.0   |
| Sodium sulfite, desiccated                                                     | gm    | 5.0   |
| Trisodium phosphate                                                            | gm    | 40.0  |
| Potassium bromide                                                              | gm    | 0.25  |
| 0.1% solution of potassium iodide                                              | cc    | 10.0  |
| Sodium hydroxide                                                               | gm    | 6.5   |
| 4-amino - N - (β-methanesulfonamidoethyl)-m-toluidinesesquisulfate monohydrate | gm    | 11.33 |
| Ethylenediamine sulfate                                                        | gm    | 7.8   |
| Citrazinic acid (2,6-dihydroxyisonicotinic acid)                               | gm    | 1.5   |

At this point it was possible to omit the conventional water wash and second hardener treatments. The film was then treated for 30 seconds at 100° F. in an acid rinse bath of the type illustrated above. The film was then washed for 1 minute in water at 100° F. and then treated for 90 seconds at 100° F. in a bleach bath having the following composition:

|                                         | Grams |
|-----------------------------------------|-------|
| Sodium ferricyanide                     | 60.0  |
| Sodium hypophosphate · H <sub>2</sub> O | 17.6  |
| Sodium bromide                          | 15.0  |
| Sodium hydroxide                        | 3.5   |
| Sodium thiocyanate                      | 5.0   |
| Water to 1 liter.                       |       |

The film was treated for 1 minute in a fixing bath having the following composition:

|                       |       |      |
|-----------------------|-------|------|
| Water 80° F. (27° C.) | liter | 1.0  |
| Sodium thiosulfate    | grams | 95.6 |
| Sodium bisulfite      | do    | 20.0 |

The film was then washed for 1 minute in 100° F. water and treated for 30 seconds in a stabilizing bath having the following composition.

|                                        |                |
|----------------------------------------|----------------|
| Constituent:                           | Fresh tank mix |
| Water                                  | ml             |
| Formalin (37.5% formaldehyde solution) | ml             |
| pH                                     |                |

It was found that improved results were obtained using the process outlined above if the concentration of sodium sulfite in the negative developer was increased to a level of about 75 grams per liter instead of the 50 grams illustrated in the example. Since conventional aldehyde hardeners could be eliminated in the process described in the example, it was found that undesired sludge and scum were easily avoided and that photographic quality remained at a high level. Also, since the film processed was harder at the start of the processing operation, considerably less dirt and suspended matter were picked up from other solutions, thus making it unnecessary to use as many wash baths as would ordinarily be employed in the processing of an unhardened film. Also, since the use of a hardened material made possible processing at a much higher temperature than normal, the hydrophilic colloid layers had much less tendency to swell in the processing solutions and made it possible to dry and film in about 1/3 the normal time. The processing time was only about 19 1/2 minutes as compared with conventional 75° F. processing which consumed about 52 1/2 minutes.

Other amine compounds can be advantageously used to obtain the unique effects illustrated in the above example. For instance, instead of using hydroxylamine to remove substantially all aldehyde from photographic material hardened in an aldehyde bath, carbohydrazide can be used to equal advantage. A typical formula which has been found useful for this purpose is as follows:

|                |       |     |
|----------------|-------|-----|
| Carbohydrazide | grams | 5   |
| Sodium sulfate | do    | 100 |
| Water to make  | liter | 1   |
| pH at 80° F.   |       | 6.0 |

The first developer, i.e., black-and-white negative developer, as employed in the above example, can be a rapid developer, such as one of the MQ type, i.e., a combination of hydroquinone and Elon developer (p-N-methylaminophenol sulfate). Other negative developers, such as hydroquinone alone, 3-pyrazolidone developers, such as 1-phenyl-3-pyrazolidone, 4,4-dimethyl-1-phenyl-3-pyrazolidone, etc., can also be used.

In order to effect color development of the photographic materials useful in our invention, any of the conventional color-forming developing agents, whose oxidation products couple with the conventional photographic cou-

plers, can be employed. Especially useful color developing agents which can be employed in our invention include aromatic primary amines containing an amino (substituted or not) or hydroxyl substituent. The phenylenediamines and substituted derivatives thereof containing a primary amino group have been found to provide excellent results in our invention. Typical of such color-forming developers are the sulfoneamido-substituted p-phenylenediamines disclosed in Weissberger U.S. Patent 2,548,574, issued April 10, 1951, the substituted p-phenylenediamines disclosed in Weissberger et al. U.S. Patent 2,566,271, issued August 28, 1951.

In the practice of the present invention, any of the conventional couplers as described in the prior art can be used. Couplers which are particularly useful in color developers include Couplers 1-64 listed in column 3-5 of Spath U.S. Patent 2,956,876, issued October 18, 1960, and also the couplers as described in the same patent in column 5 as Couplers 65-77 in which the couplers are included in the photographic silver halide emulsion layers are equally useful. Other couplers suitable for use in the emulsions of this invention include those described in Spence and Carroll U.S. Patent 2,640,776, issued June 2, 1953; Weissberger et al. U.S. Patent 2,407,210, issued September 3, 1946, and Weissberger et al. U.S. Patent 2,474,293, issued June 28, 1949. Other couplers which can be used in the emulsions of the present invention include the acylamino-substituted couplers, as disclosed in Salminen and Weissberger U.S. Patent 2,423,730, issued July 8, 1947.

The invention has been described in detail with particular reference to preferred embodiments thereof, but it will be understood that variations and modifications can be effected within the spirit and scope of the invention, as described hereinabove and as defined in the appended claims.

What we claim as our invention and desire secured by Letters Patent of the United States is:

1. A process for forming a stable image in a photographic element comprising at least one photo-exposed silver halide emulsion layer containing an organic, hydrophilic, colloid binder comprising hardening said binder by reaction with an aqueous solution of an aldehyde prior to photographic development but after photoexposure, removing substantially immediately all free aldehyde from said binder prior to any photographic development by treatment with an aqueous solution of an amine compound selected from the class consisting of (A) a primary amine selected from the class consisting of hydroxylamine, semicarbazide, hydrazine, carbohydrazide, biuret, aminoguanidine, methylsemicarbazide and water-soluble salts of said compounds and (B) Girard's reagent, developing a photographic image by treatment of said silver halide emulsion layer with an aqueous alkaline photographic developer.

2. A process for forming a stable image in a photographic element comprising at least one photo-exposed silver halide emulsion layer containing a water-permeable, organic, hydrophilic, colloid binder comprising hardening said binder by treatment with an aqueous solution of an aldehyde prior to photographic development but after photoexposure, removing substantially immediately all free aldehyde from said binder prior to any photographic development by treatment with an aqueous solution of hydroxylamine, and developing a photographic image in said silver halide emulsion layer by treatment of said silver halide emulsion layer with an aqueous alkaline photographic developer.

3. A process for forming a stable image in a photographic element comprising at least one photo-exposed silver halide emulsion layer containing a water-permeable, organic, hydrophilic, colloid binder comprising hardening said binder by treatment with an aqueous solution of an aldehyde prior to photographic development but after photoexposure, removing substantial-

ly immediately all free aldehyde from said binder prior to any photographic development by treatment with an aqueous solution of carbohydrazide, and developing a photographic image in said silver halide emulsion layer by treatment of said silver halide emulsion layer with an aqueous alkaline photographic developer.

4. A process for forming a stable image in a photographic element comprising at least one photo-exposed silver halide emulsion layer containing a water-permeable, organic, hydrophilic, colloid binder comprising hardening said binder by treatment with an aqueous solution of an aldehyde prior to photographic development but after photoexposure, removing substantially immediately all free aldehyde from said binder prior to any photographic development by treatment with an aqueous solution of semicarbazide, and developing a photographic image in said silver halide emulsion layer by treatment of said silver halide emulsion layer with an aqueous alkaline photographic developer.

5. A process for forming a stable image in a photographic element comprising at least one photo-exposed silver halide emulsion layer containing a water-permeable, organic, hydrophilic, colloid binder comprising hardening said binder by treatment with an aqueous solution of an aldehyde prior to photographic development but after photoexposure, removing substantially immediately all free aldehyde from said binder prior to any photographic development by treatment with an aqueous solution of hydrazine, and developing a photographic image in said silver halide emulsion layer by treatment of said silver halide emulsion layer with an aqueous alkaline photographic developer.

6. A process for forming a stable image in a multi-layer photographic element containing a plurality of differentially-sensitized, photo-exposed silver halide emulsion layers containing a water-permeable, organic, hydrophilic, colloid binder and a color coupler in each of said layers comprising hardening said binder by reaction with an aqueous solution of an aldehyde prior to photographic development but after photoexposure, removing substantially immediately all free aldehyde from said binder prior to any photographic development by treatment with an aqueous solution of an amine compound selected from the class consisting of (A) a primary amine selected from the class consisting of hydroxylamine, semicarbazide, hydrazine, carbohydrazide, biuret, aminoguanidine, methylsemicarbazide and water-soluble salts of said compounds and (B) Girard's reagent, and developing a photographic image by treatment of at least one of said silver halide emulsion layers with an aqueous alkaline photographic developer.

7. A process according to claim 6 wherein said amine compound is hydroxylamine.

8. A process according to claim 6 wherein said amine compound is hydrazine.

9. A process according to claim 6 wherein said amine compound is semicarbazide.

10. A process according to claim 6 wherein said amine compound is carbohydrazine.

11. In a complete photographic reversal color process wherein a multi-layer photographic element containing a plurality of differentially-sensitized, photo-exposed silver halide emulsion layers containing a water-permeable, organic, hydrophilic, colloid binder and a color coupler in each of said layers is processed in a series of baths heated to a temperature of at least 85° F. to accelerate processing, the first developing bath being a developing bath for producing a black-and-white negative image, followed by a reversal re-exposure and color development in a color developing bath, the steps of hardening the binders of said emulsion layers by treatment in an aqueous aldehyde bath prior to photographic development but after photoexposure and removing of substantially immediately all free aldehyde prior to any photographic development by treatment of said silver halide emulsion layers in an aqueous solution containing an amine compound selected from the class consisting of (A) a primary amine selected from the class consisting of hydroxylamine, semicarbazide, hydrazine, carbohydrazide, biuret, aminoguanidine, methylsemicarbazide and water-soluble salts of said compounds and (B) Girard's reagent.

12. In a process for forming a visible image in a photographic element comprising at least one photo-exposed silver halide emulsion layer containing an organic, hydrophilic, colloid binder by developing said photo-exposed layer in an aqueous alkaline photographic developer at an elevated temperature, the step comprising hardening said colloid binder by treatment with an aqueous solution of an aldehyde prior to said photographic development but after photoexposure, and removing substantially immediately all free aldehyde from said colloid binder prior to any photographic development by treatment with an aqueous solution of an amine compound selected from the class consisting of (A) a primary amine selected from the class consisting of hydroxylamine, semicarbazide, hydrazine, carbohydrazide, biuret, aminoguanidine, methylsemicarbazide and water-soluble salts of said compounds and (B) Girard's reagent.

#### References Cited by the Examiner

##### UNITED STATES PATENTS

|           |       |                 |       |          |
|-----------|-------|-----------------|-------|----------|
| 2,286,662 | 6/42  | Weyde et al.    | ----- | 96-56    |
| 2,309,492 | 1/43  | Albers et al.   | ----- | 96-22 XR |
| 2,353,690 | 7/44  | Clarkson et al. | ----- | 96-66 XR |
| 2,675,314 | 4/54  | Vettum et al.   | ----- | 96-56    |
| 2,984,567 | 5/61  | Henn et al.     | ----- | 96-22    |
| 3,113,864 | 12/63 | Yager et al.    | ----- | 96-22    |

##### FOREIGN PATENTS

|         |      |               |
|---------|------|---------------|
| 760,792 | 4/54 | Great Britain |
|---------|------|---------------|

##### OTHER REFERENCES

Glafkides: "Photographic Chemistry," vol. 1, page 150, Fountain Press, London, 1958.

NORMAN G. TORCHIN, Primary Examiner.

HAROLD N. BURSTEIN (deceased), Examiner.